

## UNITED STATES PATENT OFFICE.

JOHN W. ALDEN, OF CANTON, OHIO, ASSIGNOR TO CENTRAL ALLOY STEEL CORPORATION, OF NEW YORK, N. Y., A CORPORATION OF NEW YORK.

## WASH OR COATING FOR INGOT MOLDS.

No Drawing.

Application filed January 19, 1926. Serial No. 82,377.

The invention relates to a plastic coating or wash adapted to be sprayed or painted upon the interior of ingot molds to produce a repellent action against the splash of molten steel poured from the ladle into the mold.

The invention is particularly adapted for top pouring wherein the liquid steel or other metal is poured through a nozzle in the ladle, from a considerable height, into the mold.

10 In ordinary practice, even with the greatest care, there is a considerable splash of this molten metal against the inner walls of the ingot mold, forming pellets which quickly freeze and stick to the mold, and when the 15 molten steel rises above these pellets surface defects are thus formed upon the ingot.

It is also common for surface defects to be formed upon the ingot by waves or currents which are set up in the mold during 20 the pouring of the molten steel, these waves or currents being caused by the molten metal boiling up at one place or another as it rises in the mold and if these waves or currents adhere to the side wall of the mold, a 25 surface defect is formed on the ingot and upon the resultant billet or bloom. All such surface defects must be chipped from the ingots, billets or blooms, this chipping requiring considerable time and expense.

30 The object of the present invention is to provide a coating or wash adapted to be applied to the interior of an ingot mold, either by a brush or spray gun, for the purpose of producing a repellent action against 35 the splash and waves or currents of the molten steel to prevent the same from sticking or freezing upon the sides of the mold and forming surface defects in the ingot or the resultant bloom or billet.

40 This wash or coating preferably consists of a mixture of commercial aluminum powder and tar with a binder and may be thinned or diluted with a sufficient amount of water to permit of the same being easily applied 45 to the interior surface of the mold by a brush or spray gun.

The preferred proportions and manner of preparing the coating or wash consists in mixing seven parts of commercial aluminum 50 powder, three parts of commercial molasses, or sodium silicate, kerosene, or other binder

suitable for the aluminum powder in suitable proportion and seven parts of water. This mixture is steamed and mixed thoroughly until it assumes an appearance similar to mercury after which five parts of melted tar is added and the mixture stirred until the ingredients are thoroughly mixed, the tar being held in mechanical suspension in the aqueous mixture of aluminum and molasses or other binder.

55 The above proportions may be varied to suit different conditions.

This coating or wash combines the valuable properties of aluminum and tar, the aluminum producing a repellent action to splashes of the steel and has a deoxidizing effect upon the surface of the molten steel which forms the surface of the ingot.

60 The tar produces a slight smoke as the level of the molten steel rises in the mold, forming a layer of carbon or soot upon the sides of the mold which assists in the repellent action of the splash or waves of molten metal.

65 It has been found by commercial practice that this wash or coating when properly mixed and applied to the interior of ingot molds with sufficient temperature to dry out the moisture (approximately 212° F.) and with a reasonably clean stream of molten metal it will to a great extent produce an ingot having a surface free from defects, thus 70 improving the ingot and considerably reducing the expenditure of labor and money to remove the defects.

75 I claim:

1. The herein described coating for ingot molds comprising a mixture of commercial aluminum powder and tar.

2. The herein described coating for ingot 80 molds comprising a mixture of commercial aluminum powder, tar and a suitable binder.

3. The herein described coating for ingot molds comprising a mixture of commercial aluminum, tar and molasses.

4. The herein described coating for ingot 85 molds comprising a mixture of commercial aluminum powder, tar, a suitable binder, and water.

5. The herein described coating for ingot 90 molds comprising a mixture consisting of seven parts of commercial aluminum pow-

der, three parts of molasses, seven parts of water and five parts of tar.

6. The process of producing a coating for ingot molds which consists in mixing seven parts of commercial aluminum powder, three parts of molasses and seven parts of water, steaming and mixing thoroughly until the

mixture assumes the appearance of mercury and then adding five parts of melted tar and stirring thoroughly.

In testimony that I claim the above, I have hereunto subscribed my name.

JOHN W. ALDEN.